

## UNITED STATES PATENT OFFICE

2,103,640

## PAPER MANUFACTURE

George A. Richter, Berlin, N. H., assignor to  
 Brown Company, Berlin, N. H., a corporation  
 of Maine

No Drawing. Application March 30, 1935,  
 Serial No. 13,989

4 Claims. (Cl. 91—68)

This invention relates to the manufacture of papers having the conjunctive properties of high absorbency and high wet-strength.

When paper is put to such uses as toweling, 5 napkins, diaper linings, handkerchiefs, etc., it should preferably be not only of high absorbency but also of sufficient wet-strength to resist the disintegrating action of the water or aqueous medium absorbed thereby. Within recent years, 10 it has been discovered that an absorptive paper base can be made to acquire high wet-strength while substantially retaining its absorptive capacity by thinly enveloping substantially all of its fibers with regenerated cellulose produced 15 in situ in the base from viscose or other cellulose derivative and serving to bind together the fibers. It was then discovered that an albuminous adhesive, such as glue, although of radically different chemical composition from regenerated cellulose, functions in a way similar to regenerated cellulose provided that the albumen is insolubilized or tanned by formaldehyde or its equivalent. Both regenerated cellulose and glue, 20 however, have the common property of being water-absorbing to a considerable extent; and it is evidently this property that permits water to diffuse or penetrate through the thin envelops or coatings of binder to the fibers of the paper base while at the same time performing 25 the role of binding together the fibers quite strongly and thus of resisting fiber-separation under manipulation that would bespeak rupture 30 of the base lacking the binder-reinforcement.

I have now found that despite the fact that 35 cellulose acetate is decidedly different from both regenerated cellulose and glue in that it is water-repellent, it can be incorporated to good advantage as a wet-strengthening agent into a paper base to yield a paper product of high water-absorptivity and high wet-strength and hence especially adapted for such uses as have hereinbefore 40 been mentioned. When I say that cellulose acetate is water-repellent, I mean that, unlike a dried glue film, which swells appreciably when 45 soaked in water, a dried cellulose acetate film formed from an organic solvent solution of cellulose acetate is not perceptibly affected even after prolonged immersion in water.

In producing the paper product of the present 50 invention, what I do is to start with a paper base of high porosity and absorbency and to incorporate the cellulose acetate thereinto in a state of attenuation so great that the pore or void space in the base is substantially the same as that 55 in a similar base lacking the acetate. This means

that the water-holding capacity of the base is substantially unaffected by the cellulose acetate, whereas the wet-strength of the base is greatly increased by reason of the bonding action of the cellulose acetate on the fibers. The resulting 5 paper products are substantially odorless and non-toxic. Because of the presence therein of the cellulose acetate, they present even less fire hazard than ordinary papers. If desired, the paper product of the present invention may be 10 softened as by being led into frictional or rubbing contact with the edge of a doctor blade or by being impregnated with such cellulose-softening or plasticizing agents as glycerine, ethylene 15 glycol, oils, or the like.

In producing a paper product embodying the present invention for such purposes, for instance, as toweling, the procedure may be as follows:— The absorptive paper base may be fabricated from substantially unbeaten or only lightly beaten 20 papermaking stock on a high-speed papermaking machine, as usual; and the paper may be creped while still on the machine as ordinarily and collected in rolls as it is being delivered by the machine. The paper base thus fabricated 25 may have pore or void space therein amounting to, say, 100% or more of the space occupied by the solid fibers alone. In other words, the water-holding capacity of the paper may amount roughly to 100% or more by weight of the dry 30 fibers, the particular water-holding capacity depending upon the cellulose pulp used as raw material and the conditioning treatment, for instance, the degree of preliminary beating, that it has undergone. Thus, a refined wood pulp 35 consisting essentially of alpha cellulose, such as I may advantageously employ as raw material, would under given conditioning treatment lead to a more absorptive paper base than such ordinary pulps as kraft and/or sulphite, such as I 40 may also employ. The dried creped paper base may be progressively withdrawn from a roll and passed progressively through a bath of cellulose acetate solution containing any one of the usual volatile cellulose acetate solvents, such as acetone, 45 ethyl acetate, etc. It is necessary that the cellulose acetate solution used as the impregnant for the paper base be quite dilute in order to deposit cellulose acetate in the desired highly attenuated state in the paper body, that is, without detract- 50 ing significantly from its void or interstitial space. To this end, the cellulose acetate solution constituting the bath is preferably one whose cellulose acetate concentration or strength ranges from 0.5 to 2%. Such a solution containing, 55

- for instance, acetone as the solvent, is quite thin and fluent and so penetrates the paper base quickly and substantially uniformly throughout. As the impregnated paper base leaves the bath of cellulose acetate solution, free or excess solution may be removed therefrom, as by the action of squeeze rolls, to leave only the desired limited small amount of cellulose acetate distributed substantially uniformly through the paper body. It is preferable that only about 0.5 to 2.0% of cellulose acetate, based on the dry weight of fiber, remain in the paper body in order to impart thereto the desired characteristics. The particular amount of cellulose acetate within the foregoing range that may be incorporated into the paper base for the purpose of the present invention depends upon the compactness of the base and the character of its fiber. When such base possesses considerable bulk, as much as 2% cellulose acetate, based on fiber, may be used. In the case of a less bulky base, for instance, the ordinary paper toweling, less acetate should be used, say, about 0.5 to 1.0%, based on fiber. It may be stated that a range of from 0.5 to 2.0% of cellulose acetate, based on fiber, embodies the outer limits of cellulose acetate that may appear in the paper product of the present invention. The impregnated paper sheet may then be dried as by passage through a hot air chamber or over drier drums, the particular drier employed preferably being equipped with a solvent-recovery system. The cause of the comparatively small amount of solvent present in the impregnated paper and the volatility of the solvent, drying of the impregnated paper may be effected rapidly, insomuch that it is possible to employ in a continuous process, such as described, only one large drier drum such as constitutes the dry end of a so-called Yankee papermaking machine.
- If desired, the dilute cellulose acetate solution may be applied to the paper base other than by immersion of the base therein. Thus, the solution may be spread on a face of the base or be picked up by the base from an applicator or "kissing roll" rotating partially submerged in the solution, in which case the solution because of its high fluidity penetrates quickly and substantially uniformly throughout the paper body. The amount of cellulose acetate thus introduced into the base is controlled as in the immersion and squeezing treatments already described.
- The dried impregnated product may be softened, if desired, as hereinbefore described. When softening agents are used, however, they may be added to the cellulose acetate solution so as to obviate a separate softening treatment. For instance, rather than glycerinating the dried impregnated product, glycerine may be added in appropriate amount to the impregnating cellulose acetate solution, particularly when the cellulose acetate solvent is acetone, since glycerine is compatible with acetone. Such plasticizers as tricresyl phosphate, dibutyl phthalate, etc. may also be added to the cellulose acetate solution to develop soft or emollient quality in the finished paper product. These latter plasticizers act as softeners upon both the cellulose acetate and the paper base. Oils such as castor oil do likewise.
- The rate at which water is absorbed or imbibed by the finished paper product may be increased by adding small amounts of suitable so-called wetting-out agents to the paper base or to the impregnating cellulose acetate solution. Among such agents may be mentioned "Nekal BX",

which is the sodium salt of naphthalene sulphonic acid with side chains; "Nekal A", which is the crude sodium salt of octohydro-anthracene meta-sulphonic acid; "Nekal AEM", which is a combination of "Nekal A" with methylhexalin; "Neomerpin N", which is a high molecular weight sulphonic acid; etc.

The finished impregnated paper product has substantially the creped form imparted to the paper base during the papermaking operation by reason of the fact that the organic solvent solution of cellulose acetate does not hydrate or swell the fiber as does water or an aqueous solution and, accordingly, there is very little tendency for the crepe to "pull out". Since the cellulose acetate solution is colorless, a white paper base treated as hereinbefore described is not discolored; nor does the cellulose acetate undergo any decomposition necessitating any chemical after-treatment of the impregnated paper product.

The absorptivity of the finished paper product may be increased by causing a precipitation of the cellulose acetate in the freshly impregnated paper base. Thus, rather than passing the paper base immediately after impregnation with the dilute cellulose acetate solution to a dryer, the wet, impregnated base may be treated with water, as by running it through a water bath, to cause the acetate to precipitate out of solution onto the fibers, whereupon excess water may be removed from the sheet as by squeeze rolls and the sheet then dried. Such a practice works to good advantage when the cellulose acetate solvent is, like acetone, water-miscible. The cellulose acetate solvent leached out of the sheet by the water bath may, when the bath becomes overconcentrated therewith, be recovered by distillation from the bath effluent. In such case, the fibers of the finished paper product carry minute discrete particles of cellulose acetate which perform a fiber-bonding service but do not prevent quick access of water to the individual fibers themselves.

Other water-repellent cellulose esters might be used in lieu of cellulose acetate according to the present invention, but cellulose acetate is the preferable ester, possessing the advantage of lower cost over such esters as the formate and butyrate and being without the fire and explosion hazard of the less expensive cellulose nitrate.

It is a surprising phenomenon that despite their content of water-repellent material, the paper products of the present invention have high water-holding ability. In other words, they do not tend to shed water as do so-called sized papers. While I cannot account with precision for the water-holding ability of the paper products of the present invention, it is my theory that, unlike the initially water-soluble wet-strengthening agents, namely, the regenerated cellulose and the glue, hereinbefore mentioned, which are believed to attach themselves tightly on the fiber walls and to wet all of the wall surface but nevertheless to permit water to diffuse therethrough to the fiber walls, the cellulose esters by virtue of deposition from organic solvent solutions do not become so intimately attached to the fiber walls as not to permit seepage in between them and the fiber walls and further do not "wet" or cover all the fiber surfaces. In other words, it may be the case that even though practically all of the fiber surface is thinly coated with the water-repellent cellulose ester, there are myriad micro-

scopic loci on the fiber walls that have escaped wetting by the ester and that constitute starting points for the water to hold onto the paper and to spread by capillary action into the bodies of the fibers as well as to stay in the interstitial or void space of the paper body. This does not happen when a paper base is treated with a comparatively strong solution of cellulose ester; and in terms of my theory this could not happen, 10 since the amount of cellulose ester available for coating the fiber walls and occupying the pores and interstices of the paper is so large as leave no uncoated starting points on the wall surfaces for the influx of water into and throughout the fiber 15 bodies or walls.

It might be remarked that when a cellulose acetate film is cast or set from an acetone solution, it is necessary to take certain precautions in order to avoid what is sometimes termed a 20 "milky" or "smoky" effect in the film. Indeed, it is quite difficult to produce from acetone solutions of cellulose acetate films which are perfectly transparent. The presence of small amounts of water in the solvent is responsible for 25 impairment in the transparency of the film; and, unless precaution is taken to exclude water from the acetone solvent, residual traces of water in the film will spoil its transparency. Undoubtedly, the acetone evaporates more rapidly than 30 the water and as the last traces of water are expelled from the cellulose acetate film, there is a "crazing" action on the film, which is very apparent. So far as I have been able to ascertain, when a very dilute cellulose acetate solution is 35 applied to a porous paper sheet, as hereinbefore described, and when the solvent, for instance, the acetone, is evaporated, there is no continuous film of acetate deposited in the sheet but only multitudinous partly connected cellulose acetate particles between which there is a 40 definite lack of the kind of continuity that exists in a cellulose acetate film. This is particularly true if the paper base is treated with the dilute cellulose acetate solution in the presence of a 45 small amount of moisture, that is, when the base sheet carries moisture therein and/or when the cellulose acetate solution itself is not completely anhydrous but carries a small amount of water dispersed or dissolved therein. Accordingly, it 50 may be distinctly desirable in accordance with the present invention to treat the paper base while it contains a small percentage of moisture, say, about 5 to 12% of moisture and/or to use as the treating solution a dilute cellulose acetate solution containing, say, about 2% to 5% of water 55 dissolved or dispersed in the volatile organic solvent solution, for instance, an acetone solution of cellulose acetate containing such percentage of water dissolved therein.

I claim:—

1. A water-absorbing paper product of high wet-strength comprising a highly porous paper body and containing substantially uniformly distributed therethrough a water-repellent cellulose ester in the amount of about 0.5% to 2.0%, based on the dry weight of the paper body, deposited in said body from organic solvent solution in an attenuated and discontinuous film such that water brought into contact with said 10 paper product spreads by capillary action to the bodies of the fibers as well as entering the pores and interstices in said paper body.

2. A water-absorbing paper product of high wet-strength comprising a highly porous body 15 and containing substantially uniformly distributed therethrough cellulose acetate in the amount of about 0.5% to 2.0%, based on the dry weight of the paper body, deposited in said 20 paper body from organic solvent solution in an attenuated and discontinuous film such that water brought into contact with said paper product spreads by capillary action to the bodies of the fibers as well as entering the pores and interstices 25 in said paper body.

3. A method of producing a water-absorbing paper product of high wet-strength, which comprises impregnating a highly porous paper body substantially uniformly throughout with a dilute organic solvent solution of a water-repellent 30 cellulose ester in such amount as to incorporate into said body about 0.5% to 2.0% of said cellulose ester, based on the dry weight of said paper body, and removing the organic solvent from the impregnated paper body and depositing said 35 cellulose ester therein from solution in an attenuated and discontinuous film such that water brought into contact with the resulting paper product spreads by capillary action to the bodies 40 of the fibers as well as entering the pores and interstices in said paper body.

4. A method of producing a water-absorbing paper product of high wet-strength, which comprises impregnating a highly porous paper body substantially uniformly throughout with a dilute organic solvent solution of cellulose acetate in such amount as to incorporate into said body about 0.5% to 2.0% of cellulose acetate, based 45 on the dry weight of said paper body, and removing the organic solvent from the impregnated paper body and depositing said cellulose acetate therein from solution in an attenuated and discontinuous film such that water brought 50 into contact with the resulting paper product spreads by capillary action to the bodies of the fibers as well as entering the pores and interstices 55 in said paper body.

GEORGE A. RICHTER.